

# UNITED STATES PATENT OFFICE.

ISAAC T. DYER, OF CHICAGO, ILLINOIS, ASSIGNOR OF TWO-THIRDS TO PETER FISH AND OSCAR FITZ CLIFFORD, BOTH OF SAME PLACE.

## COMPOSITION FOR COATING IRON AND WOOD.

SPECIFICATION forming part of Letters Patent No. 425,412, dated April 15, 1890.

Application filed October 13, 1888. Renewed July 26, 1889. Serial No. 318,730. (Specimens.)

*To all whom it may concern:*

Be it known that I, ISAAC T. DYER, a citizen of the United States, and a resident of Chicago, in the county of Cook and State of Illinois, have invented new and useful Improvements in Composition for Coating Iron and Wood, of which the following is a specification, reference being had to the ingredients composing the coating and the method of compounding them and applying the same for use, as hereinafter fully set forth.

First, the purpose of this invention is to coat iron and other metals, so that salts, acids, or alkalies will not come in contact with their surfaces, by simple and comparatively inexpensive means; second, to render wood impervious to moisture and to acids and alkalies. This I accomplish by a composition made of asphaltum, lamp-black, sulphur, and lard-oil or a like oleaginous substance.

It has been the custom to coat pipes made of metal and to coat wood with asphaltum and to use lamp-black as an ingredient of paint; but a coating made of the ingredients named is original with me, and was not known before my invention thereof. Asphaltum employed alone as a coating is too porous to exclude water for a great length of time—that is, so thick a coat of asphaltum on a pipe as to exclude water is impracticable, and for excluding salts, acids, and alkalies such a coat as can be conveniently applied is of no practical use.

I make a coating which serves well the purpose of resisting these substances by filling the pores of the asphaltum with lamp-black and finely-ground sulphur. The medium employed to accomplish this is lard-oil as the cheapest and best. I take five pounds of solid asphaltum, melted in a suitable vessel, and bring it to a heat less than that which will produce combustion, add one quart of lard-oil and also add one-half pound of sulphur and one-half pound of lamp-black and incorporate the same by stirring the mass thoroughly and adding lard-oil to keep the

compound about the consistence of thick paint. This must be done where there is free ventilation, or a suction-fan must be operated over the mixing-tank to carry off the 50 fumes of sulphur, which at first are disagreeable; but they soon pass off as the mixing progresses. The composition should then stand for four to six hours, and is afterward suitable for use.

In practice a large tank of the composition can be prepared at a time and the metal or wood in a heated state can be immersed therein, or the composition in a heated condition less than to produce combustion can 60 be applied in any of the well-known ways for coating pipes or surfaces of iron and wood. By heating the material to be coated to a degree less than to produce combustion of the composition a much better protection will be 65 attained.

From time to time during the heating and stirring process it will be necessary to test the composition to find if all those portions of the oil which will not form a chemical 70 union with the other ingredients have been eliminated. This can be done by applying some of the mass to a warm iron and letting it cool. Then if the coat is hard and firm the composition is fit for use. Otherwise the 75 heating and stirring process should be continued till the composition will be hard when cool.

The composition thus prepared can be kept in a plastic form in tight casks and shipped to 80 any desired place for use.

I claim as new and desire to secure by Letters Patent of the United States—

A composition for coating metal and wood, consisting of asphaltum, sulphur, lamp-black, 85 and lard-oil, compounded substantially in the proportions given, and for the purpose specified.

ISAAC T. DYER.

Witnesses:  
G. L. CHAPIN,  
PETER FISH.